# EUROPEAN PATENT SPECIFICATION

(11) **EP 3 645 303 B1**
(45) Date of publication and mention of the grant of the patent: **29.07.2020**
(21) Application number: 19730960.2
(22) Date of filing: 20.05.2019
(51) Int. Cl.: B44C 1/17, B41M 3/12

(54) **THERMOADHESIVE LABEL WITH EMBOSSED GRAPHIC EFFECTS AND A METHOD FOR MANUFACTURING THE SAME**
THERMOADHÄSIVES ETIKETT MIT GEPRÄGTEN GRAPHISCHEN EFFEKTEN UND EIN VERFAHREN ZU DESSEN HERSTELLUNG
ÉTIQUETTE THERMOADHÉSIVE À EFFETS GRAPHIQUES EN RELIEF ET PROCÉDÉ DE FABRICATION ASSOCIÉ

(30) Priority: 23.05.2018 IT 201800005618
(43) Date of publication of application: 06.05.2020
(73) Proprietor: Stilscreen S.r.l., 20882 Bellusco (Monza Brianza) (IT)
(72) Inventor: ACATTI, Milena, 20060 Trezzano Rosa (Milano) (IT)
(74) Representative: Zermani, Umberto
(86) International application number: PCT/IB2019/054142
(87) International publication number: WO 2019/224692

(56) References cited:
- WO-A1-2016/077169
- US-B2- 6 543 810

## Description

The present invention relates to a thermoadhesive label with embossed graphic effects, as well as a method for the manufacturing of the same.

The present invention therefore finds its main application in the clothing industry, mainly of the sport type, in particular in the application of labels provided with informative shapes or contents, such as for example crests, symbols, numbers or writings.

In the known art, labels have long been known which, to facilitate fixing the same to the fabric, are provided with an adhesive able to allow adhesion by the transfer following a contextual application of pressure and heat, without the need for stitching; such labels are known as thermoadhesive or transferable labels.

In this regard, in recent years the market has increasingly shown the need to have labels that are not only easily weldable, but that from an aesthetic point of view create special and distinctive effects.

To this end, for some time now, an imprinting station has been introduced in the label manufacturing processes which, by means of appropriately engraved drums and due to the pressure of the drum, recreate on a support a predetermined graphic or texture effect, subsequently taken up by the polymeric layer of transfer.

This solution, in addition to having limitations linked to the difficulty of transferring particularly complicated textures, has considerable critical aspects in terms of flexibility.

In fact, the need to machine metal drums with the desired pattern results in the manufacturer remaining bound to the use of such graphic/texture effect for a very large number of pieces, in order to be able to absorb the machining costs of the drum.

Moreover, regardless of the technique with which the embossings are generated on the support layer, the methods for the manufacturing of the labels known up to know provide for the execution of long and expensive processes, not compatible with the requirements of a demanding market both in terms of numbers and of costs.

The object of the present invention is therefore to provide a thermoadhesive label and a method of manufacturing of said particularly efficient and economical thermoadhesive label.

Said objects are achieved by a thermoadhesive label having the technical characteristics of one or more of the subsequent claims from 1 to 4, as well as by a method of manufacturing of a thermoadhesive label having the technical characteristics listed in one or more of the claims from 5 to 11.

In particular, the thermoadhesive label with embossed graphic effects comprises a support element provided with a first face, substantially flat, and a second face having an embossed portion having a predetermined pattern in order to define, on said second face, an alternation of depressions and bulges. According to an aspect of the invention the embossed portion is made of a catalysed silicon material.

In fact, the label also comprises a transferable element provided with:
a graphic portion provided with at least one polymeric layer printed directly onto the second face of said support element and counter-shaped to it to cover its bulges and fill its depressions, and
an adhesive portion provided with at least one adhesive layer.
WO 2016/077169 A1 discloses a thermoadhesive label according to the preamble of claim 1 and a corresponding manufacturing method.

According to the characterizing aspect of the invention, the polymeric layer is made of dried single-component polyurethane resin, non-catalysed and non cross-linked.

Advantageously, the absence of cross-linking makes the transfer softer and emphasizes the tactile perceptibility of the texture.

According to the above, the method of manufacturing of the thermoadhesive label, also object of the invention, provides for the manufacturing of the support element by means of:
the provision of a base body provided with a first face and a second face,
a silk-screen printing step of a predetermined pattern on said second face of the base body, made with a silicon ink provided with a catalysing agent so as to realize, on said second face, an alternation of depressions and bulges, and
a drying and catalysing step of said silicon ink, carried out at a temperature higher than 120°C.

The method then provides to realize the graphic portion of the transferable element on the support element.

This step provides for:
at least one silk-screen printing step of at least one single-component polyurethane resin, free of catalysing and cross-linking agents, on the second face of the base body, so as to realize a polymeric layer covering its bulges and filling its depressions, and
at least one drying step, carried out at a temperature between 60 and 110°C.

At least, a manufacturing of an adhesive portion of the transferable element by means of a printing step of a thermoadhesive resin on said graphic portion of the transferable element is provided.

Advantageously, due to the presence of the silicone embossed portion it is possible to realize various types of textures simply by changing the print pattern.

Moreover, thanks to the presence of the catalysed silicone resin it is possible to deal with the need to introduce separating agents between the support element and the transferable element.

Preferably, the silk-screen printing step of at least one single-component polyurethane resin free of catalysing agents and cross-linking agents provides to print on the second face of the base body a pre-polymerized single-component polyurethane resin dissolved in a solvent; the drying step therefore provides an evaporation of said solvent such as to harden said single-component polyurethane resin.

Advantageously, the Applicant has noticed that the use of pre-polymerized monocomponent polyurethane resins and free of any cross-linking agent (as well as of catalysing agents) allows to speed up, simplify and, above all, make the production process more economical, while allowing to obtain a thermoadhesive label with excellent performance features.

In particular, the absence of cross-linking agents within the polymeric layers of the transferable element allows:
- to reduce the chemical components inside the label, simplifying success in chemical compatibility tests required by the regulations;
- to considerably increase the useful life of the stocked polyurethane resin, since the absence of a cross-linking agent makes the material usable even after some time;
- to facilitate the printing process, reducing the need for "environmental" control;
- to speed up the printing process, given the absence of a cross-linking step.

In particular, it is emphasized that the use of a solvent-based polyurethane resin, wherein the solvent evaporates completely during drying, is highly appreciable by customers also in terms of ecological compatibility.

Further features, with the related benefits, will become more apparent from the following exemplary, and therefore non-limiting, description of a preferred, and therefore not exclusive, embodiment of a thermoadhesive label with embossed graphic effects and a method for the manufacturing of the same according what illustrated in the appended figures, wherein:
- figure 1 shows a schematic cross-sectional view of a thermoadhesive label with embossed graphic effects according to the present invention;
- figure 2 shows the label of figure 1 upon the application on a fabric T;
- figures 3a-3h schematically show a succession of steps of a method for the manufacturing of the label of figure 1;
- figures 4a-4b show a schematic exploded and plan view of a thermoadhesive label with embossed graphic effects according to a further embodiment of the invention.

With reference to the appended figures, number 1 indicates a thermoadhesive label according to the present invention.

The term "thermoadhesive label" is therefore intended to define a multilayer polymeric support, having a predetermined shape and graphic characterization, which can be applied to a fabric T (or other medium) by using pressure and heat, to example by means of the use of an iron or similar industrial device (e.g. heated plates).

Such labels find application, as already mentioned initially, in the clothing sector, preferably of a sports type, mainly with the aim of allowing the application of numbers, symbols and sponsorships of different kinds on media such as sweaters, bags, teams, associations or sport clubs accessories.

The thermoadhesive label 1 is of the type provided with an embossed graphic effect, or a tactile and/or visual texture, and comprises at least one support element 2 and a transferable element 3 (or transfer).

The support element 2 therefore defines the base which, upon the transfer on the tissue T, is discarded.

The transferable element 3 is instead the actual label which, as a result of the application of pressure and heat, is transferred onto the fabric bringing therewith a predetermined shape, a predetermined graphic layout and a predetermined pattern or texture.

Note that, in the present text, with the expression "pattern" reference is made not so much to the graphic/chromatic conformation of label 1, as much to its texture, i.e. to the graphic effect generated due to the appropriate distribution of embossings and recesses that vary the brightness and of the label with the same incidence angle of a bright radiation.

The method of manufacturing of the label therefore provides for the preliminary manufacturing of the support element 2.

In particular, a base body 4 provided with a first face 4a and a second face 4b is provided. These faces 4a, 4b are both flat.

Preferably, the base body 4 is a sheet made of polymeric material, more preferably a polyester.

In the preferred embodiment, the base body 4 is made of polyethylene terephthalate (PET).

Subsequently, a silk-screen printing step of a predetermined pattern is provided on the second face 4b of the base body 4.

This printing is carried out with a layer of silicon ink 6 provided with a catalysing agent so as to realize, on said second face 4b, an embossed portion 5 provided with an alternation of depressions 5a and bulges 5b. Preferably, the printing step is performed in an environment with a stable temperature, preferably not above a predetermined maximum limit (more preferably about 24°C).

It should be noted that the thickness of the layer of silicon ink is variable depending on the desired depth for the printed pattern, the more visible and three-dimensional the greater the depth of the depressions 5a with respect to the bulges 5b.

It should be noted that, preferably, the silicon ink is further provided or associated with a cross-linking agent (immersed in a base, for example a solvent).

In this regard, upon the deposition of the silicon ink, a cross-linking step of the same is provided on the base body 2.

More preferably, the silicon ink is also mixed with a catalysing agent. Advantageously, in this way the embossed portion 5 has an increased hardness, which will be useful in the subsequent steps of the method. This step is performed upstream or simultaneously with a drying step of the support element 2, carried out in a suitable oven at a temperature above 120°C, preferably of about 140°C.

More precisely, such drying (or desiccation) step is performed in hot air ovens and insulated flat carpet, with the final part arranged for carrying out a cooling at room temperature.

The drying time is preferably between 1 minute and 2 minutes, more preferably about one and a half minutes, in order to allow a perfect stabilization of the silicone.

Therefore, upon the drying step, a support element 2 is available, provided with a first face 2a substantially flat, and a second face 2b having an embossed portion 5 defining the aforementioned "predetermined pattern". The first face 2a of the support element corresponds to the first face 4a of the base body 4.

The second face 2a of the support element 2 corresponds instead to the second face 4b of the base body 4 coated with the layer of silicon ink 6 cross-linked (and catalysed) to define the embossed portion 5 thereof. Note that the "predetermined pattern" corresponds to the negative of the graphic effect that will be visible on the transferable element 3 once applied to the fabric.

In this regard, once the support element 2 has been realized, the transferable element 3 is realized.

The transferable element 3 comprises a graphic portion 3a and an adhesive portion 3b overlapped therebetween.

In particular, the graphic portion 3a is interposed between the support element 2 and the adhesive portion 3b.

The manufacturing of the graphic portion 3a of the transferable element 3 provides in the first instance for a manufacturing/depositing step of a polymeric layer 7 on said second face 2b of the support element 2.

Such at least a polymeric layer 7 is printed directly onto the second face 2b of said support element 2 and counter-shaped to it to cover its bulges 5b and fill its depressions 5a.

According to the invention, such polymeric layer 7 is made of dried single-component polyurethane resin, non-catalysed and non cross-linked.

Advantageously, the absence of cross-linking makes the transfer softer and emphasizes the tactile perceptibility of the texture.

Moreover, in this way it is possible to speed up, simplify and, above all, make the label 1 production process more economical.

Moreover, the reversibility of the non cross-linked polymers allows to recover the resin upon the action of a solvent, resulting in a high ecological compatibility.

In this regard, therefore, the method provides at least one silk-screen printing step of at least one single-component polyurethane resin, free of catalysing agents and cross-linking agents, on the second face 4b of the base body 4 (i.e. on the second face 2b of the support element 2). Preferably, the single-component polyurethane resin is pre-polymerized and dissolved in a solvent (or solvent based).

In this way it is possible to precisely realize the polymeric layer 7, covering the bulges and filling the depressions defined by the embossed portion 5. Upon such printing a drying step is provided, carried out at a temperature between 60 and 110°C.

This drying step, therefore, evaporates the solvent and hardens the single-component polyurethane resin.

It should be noted that, at the end of drying, the embossed portion 5 has greater hardness than the polymeric layer 7.

In the preferred embodiment, the graphic portion 3a of the transferable element is multilayer.

Therefore, preferably, the silk-screen printing steps of the polyurethane resin and the drying step mentioned above are repeated several times so as to differentiate in appearance and function a plurality of different layers defining the graphic portion 3a.

In the preferred embodiment, the graphic portion 3 comprises a protective polymeric layer 8 and one or more coloured polymeric layers 9. Preferably, the protective polymeric layer 8 is printed directly on the support element 2, while the coloured polymeric layers 9 are printed, in succession, on the protective polymeric layer 8.

In particular, the protective polymeric layer 8 is made of a polyurethane resin printed directly on the second face 2a of the support element 2 and provided with said alternation of depressions 8a and bulges 8b corresponding to those of the support element.

In other words, the protective polymeric layer 8 develops between two faces, one in contact with the support element 2 and one distal from it, both of which are crimped and counter-shaped to the second face 2b of the support element 2.

More precisely, the manufacturing of the protective polymeric layer 8 provides for a first silk-screen printing step of at least one single-component transparent polyurethane resin and free of catalysing agents and cross-linking agents.

According to what stated above, preferably such transparent polyurethane resin is pre-polymerized and solvent based.

More preferably, the transparent polyurethane resin is a single-component aliphatic resin.

Such transparent polyurethane resin then undergoes a first drying step, carried out at a temperature between 60 and 110°C, preferably of about 90°C.

The drying step allows the solvent to evaporate and the resin to dry.

The coloured polymeric layers 9 are in turn made with a non-catalysed polyurethane resin and printed in succession so as to be overlapped on each other. Each of said coloured polymeric layers 9 is provided with a flat face 9a distal from the protective layer 8. Preferably, therefore, the first coloured polymeric layer 9, in contact with the protective polymeric layer 8, has a first face counter-shaped and attached to the protective polymeric layer 8 and a second flat face 9a.

The sequence and number of layers depend on the graphics and colouring of the transferable element; for example, in the embodiment illustrated in figure 1 there are two coloured polymeric layers 9, each carrying a respective colouring, while in the embodiment in figure 4a, 4b the coloured polymeric layers 9 are four.

One or more coloured polymeric layers 9 are realized by one or more second silk-screen printing steps of one or more coloured single-component polyurethane resins, free of catalysing agents and cross-linking agents.

Also, these resins are preferably pre-polymerized, and solvent based. More preferably, the coloured polyurethane resin is an aliphatic resin. Such second printing steps are performed so that each of said one or more coloured polymeric layers 9 is provided with a flat face 9a distal from the protective layer 8.

It should be noted that, in order to allow graphic stability, one or more corresponding second drying steps performed upon each second printing step and carried out at a temperature between 60 and 110°C, preferably of about 90°C, are provided.

Therefore, with each printing of a coloured polyurethane resin, a corresponding drying step follows. The drying step allows the solvent to evaporate and the resin to dry.

In addition, in the preferred embodiment, the graphic portion 3a of the transferable element 3 comprises a barrier layer 10 made of a non-catalysed polymeric material printed on said at least one polymeric layer 7. The barrier layer 10 is preferably realized by at least one silk-screen printing step, on said at least one polymeric layer 7, of a polymeric material mixed with carbon powder. Said polymeric material is free of catalysing agents and cross-linking agents.

Subsequently, a first new drying step, carried out at a temperature between 60 and 110°C, preferably of about 90°C is carried out.

In detail, the drying steps of the polymeric layers described up to this point provide for the use of a tunnel oven where a forced ventilation at room temperature and partial air extraction system ensures the drying of the printing and the expulsion of the vapours (e.g. Wicket oven).

The drying time is preferably greater than 90 minutes, more preferably about 2 hours.

Advantageously, the presence of the barrier layer 10 allows the transferable element 3a to be covering, which is particularly advantageous in labels designed for an application with sublimation printing.

In this regard, in the preferred embodiment, the presence of at least three barrier layers 10 overlapped on one another is provided.

Preferably, moreover, the transferable element comprises a further polymeric layer 11 interposed between said at least one polymeric layer 7 and the adhesive portion 3b.

The further polymeric layer 11 is therefore printed on the polymeric layer 7 or, depending on the embodiment, on the barrier layer 10.

Such further polymeric layer 11 is preferably made of a solvent-based elastic polyurethane, single-component resin and free of catalysing agents. It should be noted that the term "elastic" (or soft) herein is intended to define that the resin has a high modulus, preferably higher than 600 MPa.

Thus, in a first embodiment, wherein the transferable element is particularly flexible, the method provides a silk-screen printing step of at least one solvent-based elastic polyurethane, single-component resin and free of catalysing agents, on said at least one polymeric layer 7 (i.e. one of the protective polymeric layers 8 and coloured polymeric layer 9) and a subsequent drying step carried out at a temperature between 60 and 110°C, preferably about 90°C.

Preferably, in such embodiment the graphic portion 3a comprises two further polymeric layers 10 overlapped on each other, realized by means of two silk-screen printing steps of the elastic polyurethane resin performed in succession and separated by respective drying steps. Advantageously, in this way it is possible to obtain resistant transferable elements but, at the same time, easily adaptable to the textile media. Alternatively, in other more rigid embodiments, a further single polymeric layer 11 is printed directly on the barrier layer 10.

Finally, the adhesive portion 3b of the transferable element 3 is realized.

The adhesive portion 3b comprises at least one adhesive layer 12 printed on said at least one polymeric layer 7 (being the protective layer 8 or a coloured layer 9) or, preferably, on the further polymeric layer 11. Preferably, the adhesive layer 12 comprises a thermoadhesive resin.

This thermoadhesive resin is preferably realized with a mixture of polymeric particles (preferably copolyester) and solvent-based polyurethane resin.

Therefore, such layer is realized by printing said mixture and subsequently drying it in a drying step, preferably carried out at a temperature between 60 and 110°C, more preferably about 90°C.

The invention achieves the intended aims and achieves important advantages.

In fact, the manufacturing of the embossed portion by silk-screen printing of a silicon ink allows great ease in modifying the texture pattern, favouring the production flexibility and reducing the cost of manufacturing of the label.

Similarly, the manufacturing of the transferable element by overlapping only non-catalysed polymeric layers, considerably speeds up the production process.

In this regard, moreover, the absence of a cross-linking allows both to significantly reduce the consumption of resin, which, not being cross-linked, can be used for a longer period of time, and to provide a decomposable label if subjected to the action of a predetermined solvent, both of such aspect having a positive impact on the ecological compatibility of the piece.

## Claims

1. Thermoadhesive label with embossed graphic effects comprising:
- a support element (2) provided with a first face (2a), substantially flat, and a second face (2b) having an embossed portion (5) defining a predetermined pattern in order to determine, on said second face (2b), an alternation of depressions (5a) and bulges (5b); said embossed portion being made of catalysed silicon material;
- a transferable element (3) provided with:
a graphic portion (3a) provided with at least one polymeric layer (7), made of a polyurethane resin, moulded directly onto the second face (2b) of said support element (2) and counter-shaped to it to cover its bulges (5b) and fill its depressions (5a),
an adhesive portion (3b) provided with at least one adhesive layer (12);
**characterized in that** said polyurethane layer (7) is made of a dried single-component polyurethane resin which is non-catalysed and non cross-linked.

2. Thermoadhesive label according to claim 1, **characterized in that** said graphic portion (3a) of the transferable element (3) comprises a plurality of superimposed polymeric layers (7) thus divided:
- a protective polymeric layer (8) made of a polyurethane resin moulded directly on the second face (2b) of the support element (2) and provided with said alternation of depressions and bulges;
- one or more coloured polymeric layers (9) made of a polyurethane resin and moulded in succession so as to be overlapped, wherein each of said coloured polymeric layers (9) is provided with a flat face (9a) distal from the protective polymeric layer (8); said protective polymeric layer (8) and said one or more coloured polymeric layers (9) being all made of non-catalysed and dried single-component polyurethane resin.

3. Thermoadhesive label according to claim 1 or 2, **characterized in that** said graphic portion (3a) of the transferable element (3) comprises a barrier layer (10) made of non-catalysed polymeric material printed on said at least one polymeric layer (7).

4. Thermoadhesive label according to any of the previous claims, **characterized in that** said graphic portion (3a) of the transferable element (3) comprises a further polymeric layer (11) interposed between said at least one polymeric layer (7) and said adhesive layer (12), preferably between said barrier layer (10) and said adhesive layer (12).

5. Method for the manufacturing of a thermoadhesive label with embossed graphic effects provided with a support element (2) and a transferable element (3); said method comprising the steps of:
- manufacturing of the support element (3) by means of
provision of a base body (4) provided with a first face (4a) and a second face (4b);
a silk-screen printing step of a predetermined pattern on said second face (4b) of the base body (4), made with a layer of silicon ink (6) provided with a catalysing agent so as to realize, on said second face (4b), an alternation of depressions (5a) and bulges (5b);
a drying and catalysing step of said silicon ink (6), carried out at a temperature higher than 120°C;
- manufacturing of a graphic portion (3a) of the transferable element (3) by means of
at least one silk-screen printing step of at least one single-component polyurethane resin, free of catalysing agents and cross-linking agents, on the second face (4b) of the base body (4), so as to realize a polymeric layer (7) covering its bulges (5b) and filling its depressions (5a);
at least one drying step, carried out at a temperature between 60 and 110°C;
- manufacturing of an adhesive portion (3b) of the transferable element (3) by means of a printing step of a thermoadhesive resin on said graphic portion (3b) of the transferable element (3).

6. Method according to claim 5, **characterized in that** said step of silk-screen printing at least one single-component polyurethane resin free of catalysing agents and cross-linking agents comprises printing on the second face (4b) of the base body (4) a pre-polymerized single-component polyurethane resin which is dissolved in a solvent; said drying step causing an evaporation of said solvent and a hardening of the single-component polyurethane resin.

7. Method according to claim 5 or 6, **characterized in that** said at least one silk-screen printing step in the manufacturing of the graphic portion (3a) comprises:
- a first silk-screen printing step of at least one transparent polyurethane resin so as to provide a protective polymeric layer (8) provided with said alternation of depressions (5a) and bulges (5b);
- a first drying step, carried out at a temperature between 60 and 110°C, preferably of about 90°C;
- one or more second silk-screen printing steps of one or more coloured polyurethane resins, carried out so as to produce one or more coloured polymeric layers (9) each provided with a flat face (9a) distal from the protective layer (8);
- one or more corresponding second drying steps carried out following each second printing step and carried out at a temperature between 60 and 110°C, preferably of about 90°C,
wherein said transparent and coloured polyurethane resins are solvent based single component resins free from catalysing agents and cross-linking agents.

8. Method according any of claims from 5 to 7, **characterized in that** the manufacturing of a graphic portion (3a) of the transferable element (3) comprises:
a silk-screen printing step of at least one solvent-based elastic polyurethane, single-component resin, free of catalysing agents and cross-linking agents,
a drying step, carried out at a temperature between 60 and 110°C, so as to cause evaporation of the solvent and hardening of the polyurethane resin.

9. Method according to claim 8, **characterized in that** it comprises two silk-screen printing steps of said one elastic polyurethane resin carried out in succession with respective drying steps between one and the other.

10. Method according to any one of claims from 5 to 9, **characterized in that** said step of manufacturing of a graphic portion (3a) of the transferable element (3) further comprises:
at least one silk-screen printing step of a barrier layer (11), made of a polymeric material on said at least one polymeric layer (7), wherein said polymeric material is mixed with carbon powder and free of catalysing agents and of cross-linking agents;
a drying step, carried out at a temperature between 60 and 110°C.

11. Method according to claim 10, **characterized in that** it comprises at least three silk-screen printing steps of said barrier layer (11).

## Patentansprüche

1. Thermoadhäsives Etikett mit geprägten graphischen Effekten, umfassend:
- ein Stützelement (2), das mit einer ersten Fläche (2a), die im Wesentlichen flach ist, und einer zweiten Fläche (2b) versehen ist, aufweisend einen geprägten Abschnitt (5), der ein vorbestimmtes Muster definiert, um auf der zweiten Fläche (2b), einen Wechsel von Vertiefungen (5a) und Wölbungen (5b) zu bestimmen; wobei der geprägte Abschnitt aus katalysiertem Siliziummaterial besteht;
- ein übertragbares Element (3) versehen mit:
einem grafischen Abschnitt (3a), der mit mindestens einer Polymerschicht (7) versehen ist, die aus einem Polyurethanharz besteht, direkt auf die zweite Fläche (2b) des Stützelements (2) geformt und zu ihr gegengeformt ist, um deren Wölbungen (5b) zu bedecken und deren Vertiefungen (5a) zu füllen,
einen Klebeabschnitt (3b), der mit mindestens einer Klebeschicht (12) versehen ist;
**dadurch gekennzeichnet, dass** die Polyurethanschicht (7) aus einem getrockneten einkomponentigen Polyurethanharz besteht, das nicht katalysiert und nicht vernetzt ist.

2. Thermoadhäsives Etikett nach Anspruch 1, **dadurch gekennzeichnet, dass** der grafische Abschnitt (3a) des übertragbaren Elements (3) eine Vielzahl an überlagerten Polymerschichten (7) umfasst, die so unterteilt sind:
- eine Schutzpolymerschicht (8) bestehend aus einem Polyurethanharz, das direkt auf der zweiten Fläche (2b) des Stützelements (2) geformt und mit dem Wechsel von Vertiefungen und Wölbungen versehen ist;
- eine oder mehrere farbige Polymerschichten (9), die aus einem Polyurethanharz bestehen und nacheinander so geformt sind, dass sie überlappen, wobei eine jede der farbigen Polymerschichten (9) mit einer flachen Fläche (9a) versehen ist, die von der Schutzpolymerschicht (8) distal ist; wobei die Schutzpolymerschicht (8) und die eine oder mehrere farbige Polymerschichten (9) alle aus nicht katalysiertem und getrocknetem einkomponentigen Polyurethanharz bestehen.

3. Thermoadhäsives Etikett nach Anspruch 1 oder 2, **dadurch gekennzeichnet, dass** der grafische Abschnitt (3a) des übertragbaren Elements (3) eine Barriereschicht (10) bestehend aus nicht katalysiertem Polymermaterial umfasst, die auf die mindestens eine Polymerschicht (7) gedruckt ist.

4. Thermoadhäsives Etikett nach einem der vorhergehenden Ansprüche, **dadurch gekennzeichnet, dass** der grafische Abschnitt (3a) des übertragbaren Elements (3) eine weitere Polymerschicht (11) umfasst, die zwischen der mindestens einen Polymerschicht (7) und der Klebeschicht (12), vorzugsweise zwischen der Barriereschicht (10) und der Klebeschicht (12) angeordnet ist.

5. Verfahren zur Herstellung eines thermoadhäsiven Etiketts mit geprägten grafischen Effekten, das mit einem Stützelement (2) und einem übertragbaren Element (3) versehen ist; wobei das Verfahren die Schritte umfasst zum:
- Herstellen des Stützelements (3) mittels der Bereitstellung eines Grundkörpers (4), der mit einer ersten Fläche (4a) und einer zweiten Fläche (4b) versehen ist;
einen Siebdruckschritt eines vorbestimmten Musters auf der zweiten Fläche (4b) des Grundkörpers (4), hergestellt mit einer Schicht aus Siliziumtinte (6), die mit einem Katalysationsmittel versehen ist, um auf der zweiten Fläche (4b) einen Wechsel von Vertiefungen (5a) und Wölbungen (5b) zu realisieren;
einen Trocknungs- und Katalysierungsschritt der Siliziumtinte (6), der bei einer Temperatur höher als 120 °C durchgeführt wird;
- Herstellen eines grafischen Abschnitts (3a) des übertragbaren Elements (3) mittels
mindestens eines Siebdruckschritts von mindestens einem einkomponentigen Polyurethanharz, das frei von Katalysationsmitteln und Vernetzungsmitteln ist, auf der zweiten Fläche (4b) des Grundkörpers (4), um eine Polymerschicht (7) zu realisieren, die deren Wölbungen (5b) bedeckt und deren Vertiefungen (5a) füllt; mindestens ein Trocknungsschritt, durchgeführt bei einer Temperatur zwischen 60 und 110 °C;
- Herstellen eines Klebeabschnitts (3b) des übertragbaren Elements (3) mittels eines Druckschritts eines thermoadhäsiven Harzes auf dem grafischen Abschnitt (3b) des übertragbaren Elements (3).

6. Verfahren nach Anspruch 5, **dadurch gekennzeichnet, dass** der Schritt zum Siebdrucken mindestens eines einkomponentingen Polyurethanharzes, das frei von Katalysationsmitteln und Vernetzungsmitteln ist, das Bedrucken auf der zweiten Fläche (4b) des Grundkörpers (4) eines vor-polymerisierten einkomponentigen Polyurethanharzes umfasst, das in einem Lösungsmittel gelöst ist; wobei der Trocknungsschritt ein Verdampfen des Lösungsmittels und ein Aushärten des einkomponentigen Polyurethanharzes bewirkt.

7. Verfahren nach Anspruch 5 oder 6, **dadurch gekennzeichnet, dass** der mindestens eine Siebdruckschritt bei der Herstellung des grafischen Abschnitts (3a) umfasst:
- einen ersten Siebdruckschritt von mindestens einem transparenten Polyurethanharz, um eine Schutzpolymerschicht (8) bereitzustellen, die mit dem Wechsel von Vertiefungen (5a) und Wölbungen (5b) versehen ist;
- einen ersten Trocknungsschritt, durchgeführt bei einer Temperatur zwischen 60 und 110 °C, vorzugsweise von etwa 90 °C;
- einen oder mehrere zweite Siebdruckschritte von einem oder mehreren farbigen Polyurethanharzen, die durchgeführt werden, um eine oder mehrere farbige Polymerschichten (9) zu erzeugen, die jeweils mit einer flachen Fläche (9a) versehen sind, die von der Schutzschicht (8) distal ist;
- einen oder mehrere entsprechende zweite Trocknungsschritte, die nach einem jeden zweiten Druckschritt durchgeführt werden und bei einer Temperatur zwischen 60 und 110 °C, vorzugsweise etwa 90 °C, durchgeführt werden,
wobei die transparenten und farbigen Polyurethanharze lösungsmittelbasierte einkomponentige Harze sind, die frei von Katalysationsmitteln und Vernetzungsmitteln sind.

8. Verfahren nach einem der Ansprüche 5 bis 7, **dadurch gekennzeichnet, dass** die Herstellung eines grafischen Abschnitts (3a) des übertragbaren Elements (3) umfasst:
ein Siebdruckschritt von mindestens einem elastischen lösungsmittelbasierten Polyurethan, einem einkomponentigen Harz, das frei von Katalysationsmitteln und Vernetzungsmitteln ist,
einen Trocknungsschritt, der bei einer Temperatur zwischen 60 und 110 °C durchgeführt wird, um ein Verdampfen des Lösungsmittels und ein Aushärten des Polyurethanharzes zu bewirken.

9. Verfahren nach Anspruch 8, **dadurch gekennzeichnet, dass** es zwei Siebdruckschritte des einen elastischen Polyurethanharzes umfasst, die nacheinander mit jeweiligen Trocknungsschritten zwischen einem und dem anderen durchgeführt werden.

10. Verfahren nach einem der Ansprüche 5 bis 9, **dadurch gekennzeichnet, dass** der Schritt zum Herstellen eines grafischen Abschnitts (3a) des übertragbaren Elements (3) umfasst:
mindestens einen Siebdruckschritt einer Barriereschicht (11) bestehend aus einem Polymermaterial auf der mindestens einen Polymerschicht (7), wobei das Polymermaterial mit Kohlenstoffpulver gemischt und frei von Katalysationsmitteln und Vernetzungsmitteln ist;
einen Trocknungsschritt, durchgeführt bei einer Temperatur zwischen 60 und 110 °C.

11. Verfahren nach Anspruch 10, **dadurch gekennzeichnet, dass** es mindestens drei Siebdruckschritte der Barriereschicht (11) umfasst.

## Revendications

1. Étiquette thermoadhésive à effets graphiques en relief comprenant :
- un élément de support (2) pourvu d'une première face (2a), substantiellement plate, et d'une seconde face (2b) comportant une partie en relief (5) définissant un motif prédéterminé afin de déterminer, sur ladite seconde face (2b), une alternance de dépressions (5a) et de renflements (5b) ; ladite partie en relief étant réalisée en matériau de silicium catalysé ;
- un élément transférable (3) pourvu de :
une partie graphique (3a) pourvue d'au moins une couche polymère (7) en résine de polyuréthane, moulée directement sur la deuxième face (2b) dudit élément de support (2) et à forme complémentaire par rapport à celui-ci pour recouvrir ses renflements (5b) et remplir ses dépressions (5a),
une partie adhésive (3b) pourvue d'au moins une couche adhésive (12) ;
**caractérisée en ce que** ladite couche de polyuréthane (7) est constituée d'une résine de polyuréthane à une composante séchée étant non catalysée et non réticulée.

2. Étiquette thermoadhésive selon la revendication 1, **caractérisée en ce que** ladite partie graphique (3a) de l'élément transférable (3) comprend une pluralité de couches polymères superposées (7) ainsi divisées :
- une couche polymère protectrice (8) en résine de polyuréthane moulée directement sur la seconde face (2b) de l'élément support (2) et pourvue de ladite alternance de dépressions et de renflements ;
- une ou plusieurs couches polymères colorées (9) constituées d'une résine de polyuréthane et moulées en succession de manière à se chevaucher, dans laquelle chacune desdites couches polymères colorées (9) est pourvue d'une face plate (9a) distale de la couche polymère protectrice (8) ; ladite couche polymère protectrice (8) et lesdites une ou plusieurs couches polymères colorées (9) étant toutes constituées de résine de polyuréthane à une composante non catalysée et séchée.

3. Étiquette thermoadhésive selon la revendication 1 ou 2, **caractérisée en ce que** ladite partie graphique (3a) de l'élément transférable (3) comprend une couche barrière (10) constitué d'un matériau polymère non catalysé imprimé sur ladite au moins une couche polymère (7) .

4. Étiquette thermoadhésive selon l'une quelconque des revendications précédentes, **caractérisée en ce que** ladite partie graphique (3a) de l'élément transférable (3) comprend une couche polymère (11) supplémentaire interposée entre ladite au moins une couche polymère (7) et ladite couche adhésive (12), de préférence entre ladite couche barrière (10) et ladite couche adhésive (12) .

5. Procédé de fabrication d'une étiquette thermoadhésive à effets graphiques en relief pourvue d'un élément de support (2) et d'un élément transférable (3) ; ledit procédé comprenant les étapes de :
- fabriquer l'élément de support (3) au moyen de la fourniture d'un corps de base (4) pourvu d'une première face (4a) et d'une seconde face (4b) ;
une étape de sérigraphie d'un motif prédéterminé sur ladite seconde face (4b) du corps de base (4), réalisée avec une couche d'encre au silicium (6) pourvue d'un agent catalyseur de manière à réaliser, sur ladite seconde face (4b), une alternance de dépressions (5a) et de renflements (5b) ;
une étape de séchage et de catalyse de ladite encre au silicium (6), effectuée à une température supérieure à 120 °C ;
- fabriquer une partie graphique (3a) de l'élément transférable (3) au moyen de
au moins une étape de sérigraphie d'au moins une résine polyuréthane à une composante, exempte d'agents catalyseurs et d'agents de réticulation, sur la seconde face (4b) du corps de base (4), de manière à réaliser une couche polymère (7) recouvrant ses renflements (5b) et remplissant ses dépressions (5a) ;
au moins une étape de séchage, effectuée à une température comprise entre 60 et 110 °C ;
- fabriquer une partie adhésive (3b) de l'élément transférable (3) au moyen d'une étape d'impression d'une résine thermoadhésive sur ladite partie graphique (3b) de l'élément transférable (3).

6. Procédé selon la revendication 5, **caractérisé en ce que** ladite étape de sérigraphie d'au moins une résine polyuréthane à une composante exempte d'agents catalyseurs et d'agents de réticulation comprend l'impression sur la seconde face (4b) du corps de base (4) d'une résine polyuréthane à une composante prépolymérisée étant dissoute dans un solvant ; ladite étape de séchage provoquant une évaporation dudit solvant et un durcissement de la résine polyuréthane à une composante.

7. Procédé selon la revendication 5 ou 6, **caractérisé en ce que** ladite au moins une étape de sérigraphie dans la fabrication de la partie graphique (3a) comprend :
- une première étape de sérigraphie d'au moins une résine de polyuréthane transparente de manière à fournir une couche polymère protectrice (8) pourvue de ladite alternance de dépressions (5a) et de renflements (5b) ;
- une première étape de séchage, effectuée à une température comprise entre 60 et 110 °C, de préférence à environ 90 °C ;
- une ou plusieurs secondes étapes de sérigraphie d'une ou de plusieurs résines de polyuréthane colorées, effectuées de manière à produire une ou plusieurs couches polymères colorées (9), chacune étant pourvue d'une face plate (9a) distale de la couche protectrice (8) ;
- une ou plusieurs secondes étapes de séchage correspondantes effectuées après chaque seconde étape d'impression et effectuées à une température comprise entre 60 et 110 °C, de préférence à environ 90 °C,
dans lequel lesdites résines de polyuréthane transparentes et colorées sont des résines à une composante à base de solvant, exemptes d'agents catalyseurs et d'agents de réticulation.

8. Procédé selon l'une quelconque des revendications de 5 à 7, **caractérisé en ce que** la fabrication d'une partie graphique (3a) de l'élément transférable (3) comprend :
une étape de sérigraphie d'au moins une résine à une composante de polyuréthane élastique à base de solvant, exempte d'agents catalyseurs et d'agents de réticulation,
une étape de séchage, effectuée à une température comprise entre 60 et 110 °C, de manière à provoquer l'évaporation du solvant et le durcissement de la résine de polyuréthane.

9. Procédé selon la revendication 8, **caractérisé en ce qu'**il comprend deux étapes de sérigraphie de ladite une résine de polyuréthane élastique réalisées en succession avec des étapes de séchage respectives entre les unes et les autres.

10. Procédé selon l'une quelconque des revendications de 5 à 9, **caractérisé en ce que** ladite étape de fabrication d'une partie graphique (3a) de l'élément transférable (3) comprend de plus :
au moins une étape de sérigraphie d'une couche barrière (11), constituée d'un matériau polymère sur ladite au moins une couche polymère (7), dans lequel ledit matériau polymère est mélangé à de la poudre de carbone et est exempt d'agents catalyseurs et d'agents de réticulation ;
une étape de séchage, effectuée à une température comprise entre 60 et 110 °C.

11. Procédé selon la revendication 10, **caractérisé en ce qu'**il comprend au moins trois étapes de sérigraphie de ladite couche barrière (11).
